# EUROPEAN PATENT APPLICATION

(11) **EP 2 128 339 A1**
(43) Date of publication of application: **02.12.2009**
(21) Application number: 08156976.6
(22) Date of filing: 27.05.2008
(51) Int. Cl.: E01C 7/35, E01C 9/00

(54) **Fibre-coated construction material**

(71) Applicant: Intron Samen Meer B.v., 6136 GV Sittard (NL); Materials Innovation Centre B.V., 2134 BE Hoofddorp (NL)
(72) Inventor: van Montfort, Joannes Louis Marie, 3680 Maaseik (BE); Breur, Hendrik Jacobus Arie, 2134 BE, Hoofddorp (NL); van der Blom, Rudy Hubertus Lucia, 6171 AB, Stein (NL)
(74) Representative: Swinkels, Bart Willem

(57) **Abstract**

The invention pertains to a construction material having at least part of its surface coated with fibres, wherein said fibres have an average thickness of less than 50 dtex, an average fibre length of less than 3 mm, and wherein a predominant part of said fibres makes an acute angle of at least 45° with the tangent of the local surface of said construction material. Related therewith, in another aspect the invention pertains to the use of such a fibrous coating layer onto construction materials, for reducing traffic noise.

## Description

### FIELD OF THE INVENTION

The invention relates to fibre-coated construction materials which are capable of reducing noise. In particular, the construction materials are road and roadside surfaces, such as asphalt pavements, and noise barriers.

### BACKGROUND OF THE INVENTION

Sound and traffic noise reduction plays an important role in the development of new silent building materials for e.g. road surfaces, noise barriers, and concrete constructions.

It is known in the art to improve noise reduction of concrete surfaces by providing the concrete with a highly porous top layer (Enhanced Porosity Concrete), and further by reinforcing the concrete with fibres, for example about 1% of 50 mm long polypropylene fibres. Moreover, it is known in the art to improve noise reduction of asphalt by introducing pores (e.g. porous asphalt).

A disadvantage of these methods is that noise reduction is only moderate, in particular over time (noise reducing effect of pores in porous asphalt is not durable) . Traffic renders the pores fouled up, thus reducing any initial noise reducing properties significantly. Also, the method can only be applied when building or renewing road surfaces, and it is difficult to treat existing roads.

Hence, in the art a need exists to improve noise reduction caused by traffic, in particular tire/road contact noise, especially over prolonged periods of time. There is also a need for providing means for reducing traffic-caused noise which can easily be applied and maintained, also to existing surfaces.

### SUMMARY OF THE INVENTION

It has now been found that coating of construction materials with specific fibres results in noise reduction. Beneficially, the fibre coating can provide for emotional design.

Without unduly restricting to any theory, the improved noise reduction properties provided for by the fibre coating are attributed largely to higher sound absorption values at specific frequencies compared to the bare construction material itself. These sound absorption properties can be modified and adjusted for specific purposes. The sound absorption properties of the fibre-coated construction materials depend on the surface properties of the construction material, such as the shape and size of the hollow spaces or pores in for instance concrete or asphalt road surfaces. Sound absorption can be optimised by selecting (1) the length of the fibres, (2) the diameter of the fibres, and (3) the orientation of the fibres. For optimal noise absorption properties, a predominant part of the fibres should be oriented about perpendicular to the surface it is coated on.

In a preferred embodiment the construction material surface has a porous top layer, wherein a significant part of the surface, including the pore area, is coated with the fibres of the present invention.

### DETAILED DESCRIPTION OF THE INVENTION

The invention thus relates to a construction material wherein at least part of its surface is coated with fibres, wherein the fibres have an average thickness of less than 50 dtex, and an average fibre length of less than 3 mm. A decitex unit, abbreviated dtex, is sometimes used to express the fineness of a yarn, and equals the mass in g per 10 km of yarn.

Moreover, it was found that acceptable noise reduction is achieved when a predominant part of the fibres makes an acute angle of at least 45° with the tangent (plane) of the surface at the point of contact. Alternatively, the fibres make an average acute angle of at least 45° with the tangent (plane) of the local surface at point of contact. Following, this angle will be referred to as the "tangent angle". Since first concern is the orientation of the fibres away from the local surface, the above values are based on the acute angle of fibre with the surface. The fibers may point in any direction away from the two-dimensional surface, provided it meets the above minimum acute angle requirement. The individual fibres need not be aligned with respect to one another.

Related therewith, in another aspect the invention pertains to the use of such a fibrous coating layer onto construction materials, for reducing traffic noise. Worded differently, the invention also pertains to a process for reducing noise produced by motorized traffic, said process comprising applying the aforementioned piles to the surface of a construction material nearby road traffic. Throughout the application, the words "noise" and "sound" are used interchangeably.

Where mention is made of "surface area", or for that matter, "local surface", it refers to the part of the construction material area exposed to sound, including the pore surface area. It is due to the pores that the surface orientation may locally differ significantly from the general construction surface. The feature of a minimum tangent angle with the local surface, i.e. minimum angle with the tangent plane of the local surface, intends to take this local curvature into account.

Noise absorption improves with increasing angle and/or with the amount of fibres oriented perpendicular. Therefore, it is preferred that at least 50 %, more preferably at least 60 %, most preferably at least 70 %, in particular at least 80 % of the fibres make a minimum acute angle of at least 45 °, preferably at least 60°, more preferably at least 70°, most preferably 80° with the tangent of the local surface it is coated on. The maximum acute angle includes the value of 90°, where the fibre is oriented perpendicular to the surface it is attached to by definition, this is the maximum angle allowed for. Throughout the application, the orientation of the fibres in accordance with the present invention is referred to as "perpendicular", ignoring the fact that deviations from a 90° tangent angle is allowed for. The high acute angles do not prevent the fibres from making contact with one another, but guarantee at least a large 'contact-free' fibre surface. However, by aligning the fibres more or less directed away from the local surface and from one another, the fibre / sound contact area is optimized.

In general, the construction material may involve all variants of road surfaces or pavements, noise barriers or acoustic fencings, and other constructions nearby road traffic, such as traffic signs, concrete constructions in shape of bridges, tunnels, road railings, fronts and roofs of houses etc. Possible construction materials which can be equipped with these fibres have surfaces comprising concrete, other stone-like materials (e.g. lime stone, gypsum), all types of asphalt, plastic composite materials, synthetic foams, sport court base materials, wood, and steel and other metals. The coating may be applied to any surface, provided that the fibres will adhere to the surface. In some cases, this may require a pre-treatment, as will be discussed further below. The coating may be applied to new and existing construction materials.

From the above list, it is especially preferred to apply the fibres to road pavement, and all other kinds of surfaces suited for motorized traffic driving, even including airport runways. The invention finds particularly good use for those construction materials having at least a porous top layer. A preferred selection thereof is road surfaces having a concrete, bitumen or asphalt top layer. A preferred example is porous asphalt or porous concrete (in Dutch often addressed as 'ZOA' or 'ZOAB'), or a variant thereof. In case of a porous top layer, it is preferred to apply the fibre coating on and in the pores, often already intended to reduce noise, as discussed in the background section. Any pre-existing noise reducing properties of the fibre-coated pores are thus further enhanced.

It is preferred to coat the construction material area exposed to ambient air (and sound) with fibres as far as possible, up to 100 % coverage. Good results in terms of noise reduction are however already obtained if the construction material is coated for at least 60 % of the surface. It is preferred to apply the fibres to at least 70 %, most preferably at least 80 % of the construction surface. Most preferably, at least 90 % of the surface is coated. It is preferred that the fibre coating covers up to 95 % of the surface area.

All sorts of fibre-forming materials may be used for coating the construction materials according to the invention. Both hydrophilic and hydrophobic polymers can be employed. The fibres are commonly composed of polyester, polyamide or polyacryl, including polyesters such as poly(ethylene) terephthalate and poly(butylene) terephthalate, polyamides represented by nylon 6, 11, 12, 66 and 610, but also polyurethane, (modified) poly(vinyl alcohol), polyalkylene such as polypolyethylene or polypropylene or modified (copolymerised) forms thereof, and rayon may be applied. Also natural originating fibres, like viscose and cellulose, can be applied. The fibres may also comprise modifications, copolymers or mixtures of the afore-mentioned types. The fiber may comprise natural materials such as viscose. Combinations may also be applied.

The fibres preferably have a thickness in the range of 0.1 - 30 dtex, more preferably 0.5 - 20 dtex. The upper limit is preferably lower than 10 dtex. These thicknesses apply to average values. A certain percentage (e.g. up to 10%) outside these ranges will not detract from the effectiveness of the fibre.

The fibre length is typically larger than 0.1 mm. In case of a porous construction material, the upper limit of the fibre length is controlled by the average size of the pores to be coated with fibres. In addition, a high fibre length and/or thickness adds surplus weight and costs. Preferably the fibre length is less than 2.5 mm, and optimally, the maximum length is less than 2 mm. The desired fibre length can be achieved by conventional means such as cutting.

It is preferred that the fibrous coating has a fibre density of 0.1 - 50 fibres/mm², preferably 0.5 - 30 fibres/mm², more preferably 1 - 20 fibre/mm², the actual numbers dependent on the fibre thickness.

In one embodiment the fibres form a fur-like coating layer, i.e. exhibiting some degree of swaying, provided the fibre coating satisfies the criterion of a more or less perpendicular orientation towards the coated surface. In other words, swaying is allowed for, provided that the above-defined acute angle with the tangent plane of the surface is met.

In another aspect the invention also pertains to a process for producing a construction material with a fibrous coating layer according to the present invention, said process comprising providing the surface of a construction material with a coat of the aforementioned piles. The piles or fibre flocks may be adhered to the construction material applying any method known in the art, provided means are taken to render the fibres perpendicular to the surface. Several methods are described in EP-A-312.600, albeit for marine applications, its contents hereby incorporated by reference.

In a preferred embodiment, the "standing" or perpendicular orientation of the fibres is achieved by charging the fibres electrostatically beforehand, prior to application. Once applied, the fibres are found to maintain their desired orientation to a large extent. Electrostatic deposition is a known phenomenon to the person skilled in the art, sometimes referred to as electrostatic flocking.

In one embodiment the fibre coating is provided to the construction material surface by first applying an adhesive, for instance an epoxy or a polyurethane, to the construction material to form an adhesive layer. The adhesive may be applied by spraying or rolling, where after the selected fibres are brought into contact with the adhesive layer, for instance using spraying techniques.

In one embodiment, the piles may also be applied as a sheet. Therefore, the invention also relates to a sheet comprising a base member and the fibres of the invention attached thereto. The base member can be made of any kind of material, e.g. polyester, polyethylene, polypropylene, vinyl, textile and paper-like materials. Such a method may especially be beneficial in cases where no direct contact with road traffic is made, such as acoustic fencing.

In another embodiment, it is possible to apply the fibres onto asphalt surface while it still exhibits viscoelastic properties, i.e. directly after formation, during road construction. In such case, adhesive may not be necessary.

A first step of providing a layer of adhesive to the object may be performed by e.g. spraying, dipping or rolling. In order to save adhesive material in case of spraying of netting, wasted adhesive may be collected below the netting. In case of dipping, care must be taken to avoid inhomogeneous layer formation, for instance using air-jetting. Foamed adhesives may be used. Also, the rheology of the adhesive can be adjusted.

The method of fabrication is adapted to the particular use of the fibres as a coating, and can be applied to surfaces. In order to achieve an evenly distributed fibre-layer, it is found useful to optimise flow potential and/or the distance between the flow outlet and the object to be covered. The fibres may also be applied in two or more steps: first a low density but evenly distributed flock of fibres is provided to the object, where after a more dense coverage is achieved with sequential flocking steps. Every step may have its own optimal velocity and outlet-object distance. It is considered to be within the skilled person's ambit to determine the optimal conditions.

As mentioned earlier, the fibre coating is applied to construction materials to achieve noise reduction, preferably traffic noise reduction, more preferably tire/road traffic noise reduction.

Traffic noise comes from a variety of sources. The engine, the powertrain, the rolling noise of the tires on the road and the noise of the wind in the vehicle body all contribute to the actual traffic noise. Depending on vehicle speed, sometimes the one, sometimes the other factor plays a bigger role. At speeds in excess of 50 km/h the traffic noise is dominated by tire/road contact noises, such as on main roads and highways. For purpose of the invention, traffic noise is simply divided between propulsion noise and tire/road contact noise, each having its own frequencies. The fibres of the invention preferably reduce both propulsion noise and tire/road contact noise. In order to achieve the latter, it is preferred to apply the fibres to the road pavement where the tire makes contact. The noise aimed for has frequencies in the range of 200 - 3000 Hz, preferably 500 - 2000 Hz. Tire/road contact noise especially concentrates in these ranges.

Within these ranges, it is preferred to increase the noise absorption coefficient on average by more than 10 %, preferably more than 15 %, most preferably more than 20 %, compared to that of the original unmuffled counterpart. The coefficient can be determined using acoustic measurements, such as laid down in the examples. The numbers in the application may be based on ISO 10534-2 (Acoustics - Determination of sound absorption coefficient and impedance in impedance tubes. Part 2: Transfer-function method).

To tackle the problem of traffic noise, it is preferred that the coating is applied to constructions which are in direct vicinity of the noise-producing traffic, preferably within a range of 50 m, preferably directly on or along traffic roads. Reference is made to the foregoing paragraph on suitable construction materials. Obviously, reducing tire/road contact noise requires direct adherence of the coating to the road exposed to traffic.

### EXAMPLES

### Example 1 - Asphalt coated with fibre flock

A piece of 20 cm x 30 cm of asphalt was covered with 3 dtex nylon fibres of 0.5 mm length by electrostatic flocking, to ensure the fibres are attached perpendicular to the surface, using a solvent based pulyurethane adhesive, which was sprayed on the asphalt. After complete drying of the adhesive, noise reduction characteristics of the fibre coated asphalt were determined as described in Example 3, and compared with untreated asphalt.

With microscopy it was revealed that the tangent angle of a predominant part of the fibres was beyond 45 °C. A microscopic picture is shown in Figure 1.

### Example 2- Asphalt coated with fibre flock

A piece of 20 cm x 30 cm of asphalt was covered with 0.9 dtex nylon fibres of 0.3 mm length by electrostatic flocking to ensure the fibres are attached perpendicular to the surface, using a solvent based polyurethane adhesive, which was sprayed on the asphalt. After complete drying of the adhesive, noise reduction characteristics of the fibre coated asphalt were determined as described in Example 3, and compared with untreated asphalt.

### Example 3 - Effect of coating on noise reduction

The acoustic effect of the fibres according to examples 1 and 2 of the invention was demonstrated as follows:

In a conditioned room (65 %RH and 20 °C) a leather ball was released at a height of 2 meters above the floor, rendering a velocity upon impact of 22.5 km/hour. The noise at impact was registered using a microphone. The results were analysed in terms of frequency.

The noise reduction of both fibre types are given in Figure 2, and compared with untreated asphalt. Clearly, the noise absorption coefficient is increased with the fibre coating.

## Claims

1. A construction material having at least part of its surface coated with fibres, wherein said fibres have an average thickness of less than 50 dtex, an average fibre length of less than 3 mm, and wherein a predominant part of said fibres makes an acute angle of at least 45° with the tangent of the local surface of said construction material.

2. The construction material according to claim 1, being road pavement or any other surface suited for motorized traffic driving.

3. The construction material according to claim 1 or 2, having a porous top layer.

4. The construction material according to claim 3, having a porous concrete, bitumen and/or asphalt top layer.

5. The construction material according to claim 1, being acoustic fencing.

6. The construction material according to any one of the preceding claims, said fibres having an average thickness ranging from 0.1 - 30 dtex.

7. The construction material according to any one of the preceding claims, said fibres having an average length ranging from 0.1 - 2.5 mm.

8. Use of a fibre coating layer onto construction material for reducing traffic noise, wherein said fibres have an average thickness of less than 50 dtex, an average fibre length of less than 3 mm, and wherein a predominant part of the fibres makes an acute angle of at least 45° with the tangent plane of the coated local surface of said construction material.

9. Use according to claim 8, said construction material being road pavement or any other surface suited for motorized traffic driving, said traffic noise being tire/road traffic noise.

10. Use according to claim 8, said construction material being acoustic fencing.

11. A process for producing a coated construction material according to any one of claims 1 - 7, said process comprising (i) providing electrostatically charged fibres having an average thickness of less than 50 dtex, and an average fibre length of less than 3 mm, and (ii) bringing said electrostatically charged fibres into contact with said construction material.
